



US008486237B2

(12) **United States Patent**  
**Krishna et al.**

(10) **Patent No.:** **US 8,486,237 B2**  
(45) **Date of Patent:** **Jul. 16, 2013**

(54) **PROCESS FOR CONTINUOUS COATING DEPOSITION AND AN APPARATUS FOR CARRYING OUT THE PROCESS**

(75) Inventors: **Lingamaneni Rama Krishna**, Hyderabad (IN); **Nitin Pandurang Wasekar**, Hyderabad (IN); **Govindan Sundararajan**, Hyderabad (IN)

(73) Assignee: **International Advanced Research Centre for Powder Metallurgy and New Materials (ARCI)**, New Delhi (IN)

(\*) Notice: Subject to any disclaimer, the term of this patent is extended or adjusted under 35 U.S.C. 154(b) by 620 days.

(21) Appl. No.: **12/579,002**

(22) Filed: **Oct. 14, 2009**

(65) **Prior Publication Data**

US 2010/0163421 A1 Jul. 1, 2010

(30) **Foreign Application Priority Data**

Oct. 16, 2008 (IN) ..... 1829/DEL/08

(51) **Int. Cl.**

*C25B 9/00* (2006.01)  
*C25D 17/00* (2006.01)  
*C25D 5/00* (2006.01)

(52) **U.S. Cl.**

USPC ..... 204/275.1; 205/137; 205/138; 205/316;  
205/333; 204/202

(58) **Field of Classification Search**  
USPC ..... 204/275.1  
See application file for complete search history.

(56) **References Cited**

U.S. PATENT DOCUMENTS

5,616,229 A 4/1997 Samsonov et al.  
5,804,053 A \* 9/1998 Vaccaro et al. ..... 205/138  
6,197,178 B1 \* 3/2001 Patel et al. ..... 205/81  
6,893,551 B2 \* 5/2005 Krishna et al. ..... 205/316

FOREIGN PATENT DOCUMENTS

IN 209817 12/2007

\* cited by examiner

*Primary Examiner* — Harry D Wilkins, III

*Assistant Examiner* — Bryan D. Ripa

(74) *Attorney, Agent, or Firm* — The Webb Law Firm

(57) **ABSTRACT**

An apparatus for continuously forming thin ceramic coatings on metal sheets, foils or wires. The apparatus has a reaction chamber, perforated nylon sheets, nylon bar guides, copper rods attached to a power supply, nylon collecting rods, and an inlet and an outlet. The reaction chamber is capable of containing an electrolytic solution. The copper rods are separately connected to the R, Y, or B phase of the power supply. Each phase is provided with two thyristors and the output of the thyristors is connected to the copper rods using current transformers. A process for continuously forming thin ceramic coatings on metal sheets, foils or wires is also provided.

**15 Claims, 2 Drawing Sheets**



FIG. 1

FIG. 2

FIG. 3

**FIG. 4**

## 1

**PROCESS FOR CONTINUOUS COATING  
DEPOSITION AND AN APPARATUS FOR  
CARRYING OUT THE PROCESS**

BACKGROUND OF THE INVENTION

1. Field of the Invention

The invention relates to a process for continuous coating deposition and an apparatus for carrying out the process. The invention more particularly relates to a process for forming oxide based ceramic coatings on reactive metal and alloy sheets, foils and wires that are in the form of a web in a continuous manner and an apparatus therefor. The films obtained according to the present invention have a glossy surface finish, thermal and electrical insulation, chemical inertness, environmental inertness, surface cleaning ability, anti-dust sticking and have good scratch resistance. Further, the process described in the present invention deposits the oxide ceramic films at a rapid rate and enhances the productivity to a great extent.

2. Description of Related Art

The metals like Al, Ti, Mg and their alloys are commercially and widely used in the engineering industries like automobile, aerospace, textile, petrochemical and crockery in the form of rods, bars, tubes, foils, sheets, wires, pipes, channels, sections, pulleys, cylinders, pistons, etc. Apart from the specific promising properties and commercial availability that these materials have, the main reason for using these materials is their high strength to weight ratio. However, there exists a limitation to use these materials beyond a certain point; the limitation arises from the fact that these materials exhibit poor resistance to wear and tear, chemical attack and heat.

Traditionally, anodizing is employed to obtain coatings on Al-alloys. But the resultant coatings are found to be porous and weakly adherent to the substrate, and thereby can not provide high level protection against wear and tear and corrosion. Moreover, coating deposition rates achieved are also low in the anodizing process.

Thermal spraying techniques like plasma spraying, high velocity oxy-fuel spraying, and detonation spraying are well developed and widely used by the engineering industry to produce large varieties of metallic, oxide, carbide and nitride based ceramic coatings. These coatings are essentially employed to combat various forms of wear and tear and corrosion and thereby enhance the service life of the components made of different metals and alloys. However, thermal spray techniques demand a high degree of pre-coating and post-coating operations that are often costly. Size, shape and complexity in geometry of the engineering components do restrict the applicability of the thermal spray techniques. Moreover, these techniques demand high quality as well as costly powders such as Alumina, Alumina-Titania, Tungsten Carbide-Cobalt, Chromium Carbide-Nickel Chrome prepared by specially developed manufacturing routes such as sol-gel, atomization, fusing, sintering and crushing, chemical reduction and blending. Deposition efficiency of these powders is always much less than 100% thus requiring a special means of unused powder separation from the coating chamber. Since these coating techniques employ spraying of heated powder particles on to relatively cold surfaces, poor metallurgical bonding between the substrate and the coating often results. These coatings are often characterized by inherent porosity, micro-cracks and higher levels of residual stresses which in turn lead to the failure of the coatings in the case of critical applications. Due to the associated coating deposition mechanism, the thermal spray techniques are not at all suitable to deposit thin films on sheets, foils and wires.

## 2

Moreover, it is not practically possible to deposit thin coatings on thin sheets, foils and wires in a continuous manner.

Yet another field of research in the area of thin film deposition on sheets, foils and wires is by means of Physical Vapor Deposition (PVD) and Chemical Vapor Deposition (CVD) techniques. However, due to the inherent nature of these processes wherein the overall coating deposition is significantly influenced by the ionic/atomic scale interactions with the surfaces being coated, the overall coating deposition rates are extremely low and production rates are very low. Besides the slow deposition nature of these processes, these techniques are also not suitable for coating deposition on a continuous scale on extremely larger/longer surface areas.

To overcome the above-mentioned difficulties and limitations and the present day need for coatings exhibiting improved tribological, electrical, thermal and chemical properties and having higher density and excellent wear resistance, research work in the area of developing an improved micro-arc oxidation process has gained importance globally.

There exist a good number of patents and publications which deal with ceramic coating deposition processes on aluminum and its alloys. Some relevant literature on prior art micro-arc processes is referred to below.

According to U.S. Pat. No. 6,197,178, a three-phase pure sinusoidal potential of 480V AC electrical power is supplied to aluminum alloy web and current densities between 20 and 70 A/dm<sup>2</sup> are applied. During the process, current density is maintained by moving the web relative to each other. An electrolyte with KOH, Na<sub>2</sub>SiO<sub>3</sub> and Na<sub>2</sub>O.Al<sub>2</sub>O<sub>3</sub>.3H<sub>2</sub>O in the proportion of 2 grams per liter of de-ionized water is used. That temperature of the electrolytic bath is maintained between 25° C. and 80° C. The coating thickness achieved is reported to be in the range of 100 to 160 microns for a 30 minute processing time on cylindrical samples.

Although the resultant coatings were found to have strong adherence with the substrate, no information is available with respect to the density and uniformity of the coatings achieved. Coating density is a very important parameter that affects the wear resistance of the resulting coatings.

In the invention cited above, the inventors used a pure sinusoidal voltage waveform without any waveform modification, while a sharply-peaked waveform makes a major contribution in providing a dense and hard coating. This is why the coatings obtained through the above-mentioned process exhibit lower hardness, i.e., 1200-1400 kg/mm<sup>2</sup>. However, there is no mention of the application of the said process to deposit coatings on thin sheets, foils and wires or to do so in a continuous manner.

U.S. Pat. No. 5,616,229 granted to Samsonov et al. discloses a method of forming a ceramic coating on valve metals. This method comprises application of at least 700V alternating current across the parts to be coated. Waveform modification is achieved through a capacitor bank connected in series between a high voltage source and the metallic body to be coated. Waveform of the electric current rises from zero to its maximum height and falls to below 40% of its maximum height within less than a quarter of a full alternating cycle.

The electrolyte used in the above cited process contains 0.5 grams/liter NaOH, 0.5-2 grams/liter KOH. In addition, the electrolyte also contains sodium tetrasilicate for which there is no claim on the exact amount to be added. During the process, the electrolyte composition is changed by adding oxyacid salt of an alkali metal in a concentration range of 2 to 200 grams per liter of solution. The process has been demonstrated by coating an aluminum alloy known as Duralumin by employing three different electrolytic baths. However, in the

process explained above there is no mention of maintaining any particular ratio between the alkali and metal silicate.

In the micro-arc oxidation process, alkali is actually responsible for dissolving the coating, whereas the metal silicate is responsible for coating buildup through poly condensation of silicate anions. Too high silicate concentration in the electrolyte causes higher coating buildup especially at sample edges rather than at other portions of the sample thus resulting in a non-uniform coating. Hence, there is a need to maintain a certain degree of proportion between the alkali and metal silicate in order to end up with uniform and dense coatings. However, there is no mention of the application of the said process to deposit coatings on thin sheets, foils and wires or to do so in a continuous manner.

In the process disclosed in U.S. Pat. No. 5,616,229 a process is described wherein an average deposition rate of 2.5 micron per minute has been achieved. However, the thickness of a fully melted inner layer is only 65 microns out of a total coating thickness of 100 microns. This indicates that this process can produce coatings comprising only 65% initial dense layer and remaining 35% external layer is porous with 4-6 pores per sq. cm. and an average pore diameter of 8-11 microns.

To make these coatings suitable for wear resistant applications, the external porous layer of sufficient thickness needs to be completely removed by machining or grinding. Apart from the fact that these machining or grinding operations are costly, machining/grinding of coated parts of complex, non-symmetric shapes is extremely difficult and demands a high degree of automated machinery and higher skill levels. This effectively increases the cost of the coating per unit volume. However, there is no mention of the application of the said process to deposit coatings on thin sheets, foils and wires or to do so in a continuous manner.

The prior art processes of micro-arc oxidation processes yielded thick dense, adherent coatings with higher coating deposition rates but failed to produce thin films on a continuous scale so as to coat several meters and kilometers long sheets or foils and wires wherein it is essentially required to impart a glossy surface finish, thermal and electrical insulation, chemical inertness, surface cleaning ability, environmental inertness, anti-dust sticking and have good scratch resistance to find potential applications in the field of decorative, insulation, anti-dust sticking applications.

Moreover, in the prior art, the processes employed for coating metallic web has been discussed in detail, but nothing has been disclosed about the general apparatus employed for carrying out the coatings on thin sheets, foils and wires or to do so in a continuous manner process in continuous scale.

According to the invention disclosed in U.S. Pat. No. 6,197,178, the apparatus employed for obtaining the coating consists of a chemically inert coating tank disposed within an outer tank. The outer tank contains heat exchange fluid. Electrolyte from the inner tank is circulated through the heat exchange disposed in the outer tank itself. To remove heat from the heat exchange fluid, heat exchange fluid is withdrawn from the outer tank with the help of a pump and then passed through a forced air cooled heat exchanger. The operation of the exchangers was controlled automatically so as to maintain the desired temperature within the electrolyte bath. However, there exists a serious drawback with this kind of setup. When a component of larger size than that of the inner coating tank is to be coated, the dimensions of the inner tank must be increased, which in turn may demand changing the outer tank dimensions as well. This makes the process more costly.

In our Indian Patent No. 209817, the following process has been described:

A process for forming coatings on bodies of reactive metals and alloys which comprises electrolysing in a non-metallic, 5 non-reactive, non-conductive reaction chamber containing an alkaline electrolytic solution having a pH>12 and conductivity>2 millimhos, comprising potassium hydroxide, sodium tetrasilicate and de-ionized or distilled water, immersing at least two metallic bodies selected from the reactive group of 10 metals on which coatings have to be effected, the bodies being fixed in a movable manner, each body being connected to an electrode, passing wave multiphase alternating current across the said bodies by thyristors connected in parallel for a period based on the desired thickness of the coating to be achieved, 15 slowly increasing the current being supplied to the said bodies until the required current density is achieved, then maintaining the current at the same level throughout the process, the electric potential being further increased gradually to compensate for the increasing resistance of the coating when the 20 visible arcing at the surface of the immersed regions of the said bodies is noticed, regulating the composition of the electrolyte by measuring its pH and conductivity during the process by conventional methods, maintaining the temperature of the electrolyte between the range of 4° C. to 50° C. and 25 keeping the electrolyte in continuous circulation throughout the process.

The patent also discloses an apparatus for carrying out the process. The apparatus disclosed in the patent is shown in FIGS. 1, 2, and 3 of the first sheet of drawings accompanying 30 this specification. In the drawings:

FIG. 1 represents a front view of a coating apparatus for carrying out the process disclosed in the prior art Indian patent;

FIG. 2 represents a front view of a main control panel for 35 carrying out the process disclosed in the patent; and

FIG. 3 represents a front view of a remote control panel for carrying out the process disclosed in the patent.

The apparatus for carrying out the process as disclosed in the patent comprises a non-metallic, non-conductive, non-reactive chamber (1) (named as reaction chamber) housing at 40 least two metallic bodies (2), the surfaces of which are to be coated, the bodies being connected to the electrical power carrying arm (3) provided with a height adjustable mechanism (4), an inlet (5) for the electrolyte provided at the bottom, and an outlet (6) at the top of the chamber, on the panel of main controller (8), analog voltmeter (9), and ammeter (10) being provided to indicate the input voltage and current, a lever type electric power on/off (11) being provided, a potentiometer (12) provided for slowly increasing the current supply to the metallic bodies (2), contractor on/off (13), thyristor on/off (14) switches, manual/automatic voltage adjustment (15), and local/remote operation (16) selector switches being 45 also provided, thyristor (not shown) and transformer (17) outputs being connected through the separate analog voltmeters (18) and ammeters (19), two separate digital temperature indicators (20) being attached to the panel of remote controller (21), the temperature of electrolyte at the inlet and outlet being measured through the thermocouples (not shown), an oscilloscope (22) attached to the remote controller (21) for 50 monitoring the electrical potential and current waveforms during the process, digital voltmeter (23) and ammeter (24) attached to the remote control panel (21) being used to monitor the changes in the current and voltage during the coating process, the height of electrolytic column (7) in the reaction chamber (1) being adjusted through a dimmerstat (25) attached to the panel of remote controller (21) and an emergency stop button (26) being attached to the remote control 55 60 65 66 67 68 69 70 71 72 73 74 75 76 77 78 79 80 81 82 83 84 85 86 87 88 89 90 91 92 93 94 95 96 97 98 99 100 101 102 103 104 105 106 107 108 109 110 111 112 113 114 115 116 117 118 119 120 121 122 123 124 125 126 127 128 129 130 131 132 133 134 135 136 137 138 139 140 141 142 143 144 145 146 147 148 149 150 151 152 153 154 155 156 157 158 159 160 161 162 163 164 165 166 167 168 169 170 171 172 173 174 175 176 177 178 179 180 181 182 183 184 185 186 187 188 189 190 191 192 193 194 195 196 197 198 199 200 201 202 203 204 205 206 207 208 209 210 211 212 213 214 215 216 217 218 219 220 221 222 223 224 225 226 227 228 229 230 231 232 233 234 235 236 237 238 239 240 241 242 243 244 245 246 247 248 249 250 251 252 253 254 255 256 257 258 259 2510 2511 2512 2513 2514 2515 2516 2517 2518 2519 2520 2521 2522 2523 2524 2525 2526 2527 2528 2529 2530 2531 2532 2533 2534 2535 2536 2537 2538 2539 2540 2541 2542 2543 2544 2545 2546 2547 2548 2549 2550 2551 2552 2553 2554 2555 2556 2557 2558 2559 25510 25511 25512 25513 25514 25515 25516 25517 25518 25519 25520 25521 25522 25523 25524 25525 25526 25527 25528 25529 25530 25531 25532 25533 25534 25535 25536 25537 25538 25539 25540 25541 25542 25543 25544 25545 25546 25547 25548 25549 255410 255411 255412 255413 255414 255415 255416 255417 255418 255419 255420 255421 255422 255423 255424 255425 255426 255427 255428 255429 255430 255431 255432 255433 255434 255435 255436 255437 255438 255439 255440 255441 255442 255443 255444 255445 255446 255447 255448 255449 255450 255451 255452 255453 255454 255455 255456 255457 255458 255459 255460 255461 255462 255463 255464 255465 255466 255467 255468 255469 255470 255471 255472 255473 255474 255475 255476 255477 255478 255479 255480 255481 255482 255483 255484 255485 255486 255487 255488 255489 255490 255491 255492 255493 255494 255495 255496 255497 255498 255499 2554100 2554101 2554102 2554103 2554104 2554105 2554106 2554107 2554108 2554109 2554110 2554111 2554112 2554113 2554114 2554115 2554116 2554117 2554118 2554119 25541100 25541101 25541102 25541103 25541104 25541105 25541106 25541107 25541108 25541109 25541110 25541111 25541112 25541113 25541114 25541115 25541116 25541117 25541118 25541119 255411100 255411101 255411102 255411103 255411104 255411105 255411106 255411107 255411108 255411109 255411110 255411111 255411112 255411113 255411114 255411115 255411116 255411117 255411118 255411119 2554111100 2554111101 2554111102 2554111103 2554111104 2554111105 2554111106 2554111107 2554111108 2554111109 2554111110 2554111111 2554111112 2554111113 2554111114 2554111115 2554111116 2554111117 2554111118 2554111119 25541111100 25541111101 25541111102 25541111103 25541111104 25541111105 25541111106 25541111107 25541111108 25541111109 25541111110 25541111111 25541111112 25541111113 25541111114 25541111115 25541111116 25541111117 25541111118 25541111119 255411111100 255411111101 255411111102 255411111103 255411111104 255411111105 255411111106 255411111107 255411111108 255411111109 255411111110 255411111111 255411111112 255411111113 255411111114 255411111115 255411111116 255411111117 255411111118 255411111119 2554111111100 2554111111101 2554111111102 2554111111103 2554111111104 2554111111105 2554111111106 2554111111107 2554111111108 2554111111109 2554111111110 2554111111111 2554111111112 2554111111113 2554111111114 2554111111115 2554111111116 2554111111117 2554111111118 2554111111119 25541111111100 25541111111101 25541111111102 25541111111103 25541111111104 25541111111105 25541111111106 25541111111107 25541111111108 25541111111109 25541111111110 25541111111111 25541111111112 25541111111113 25541111111114 25541111111115 25541111111116 25541111111117 25541111111118 25541111111119 255411111111100 255411111111101 255411111111102 255411111111103 255411111111104 255411111111105 255411111111106 255411111111107 255411111111108 255411111111109 255411111111110 255411111111111 255411111111112 255411111111113 255411111111114 255411111111115 255411111111116 255411111111117 255411111111118 255411111111119 2554111111111100 2554111111111101 2554111111111102 2554111111111103 2554111111111104 2554111111111105 2554111111111106 2554111111111107 2554111111111108 2554111111111109 2554111111111110 2554111111111111 2554111111111112 2554111111111113 2554111111111114 2554111111111115 2554111111111116 2554111111111117 2554111111111118 2554111111111119 25541111111111100 25541111111111101 25541111111111102 25541111111111103 25541111111111104 25541111111111105 25541111111111106 25541111111111107 25541111111111108 25541111111111109 25541111111111110 25541111111111111 25541111111111112 25541111111111113 25541111111111114 25541111111111115 25541111111111116 25541111111111117 25541111111111118 25541111111111119 255411111111111100 255411111111111101 255411111111111102 255411111111111103 255411111111111104 255411111111111105 255411111111111106 255411111111111107 255411111111111108 255411111111111109 255411111111111110 255411111111111111 255411111111111112 255411111111111113 255411111111111114 255411111111111115 255411111111111116 255411111111111117 255411111111111118 255411111111111119 2554111111111111100 2554111111111111101 2554111111111111102 2554111111111111103 2554111111111111104 2554111111111111105 2554111111111111106 2554111111111111107 2554111111111111108 2554111111111111109 2554111111111111110 2554111111111111111 2554111111111111112 2554111111111111113 2554111111111111114 2554111111111111115 2554111111111111116 2554111111111111117 2554111111111111118 2554111111111111119 25541111111111111100 25541111111111111101 25541111111111111102 25541111111111111103 25541111111111111104 25541111111111111105 25541111111111111106 25541111111111111107 25541111111111111108 25541111111111111109 25541111111111111110 25541111111111111111 25541111111111111112 25541111111111111113 25541111111111111114 25541111111111111115 25541111111111111116 25541111111111111117 25541111111111111118 25541111111111111119 255411111111111111100 255411111111111111101 255411111111111111102 255411111111111111103 255411111111111111104 255411111111111111105 255411111111111111106 255411111111111111107 255411111111111111108 255411111111111111109 255411111111111111110 255411111111111111111 255411111111111111112 255411111111111111113 255411111111111111114 255411111111111111115 255411111111111111116 255411111111111111117 255411111111111111118 255411111111111111119 2554111111111111111100 2554111111111111111101 2554111111111111111102 2554111111111111111103 2554111111111111111104 2554111111111111111105 2554111111111111111106 2554111111111111111107 2554111111111111111108 2554111111111111111109 2554111111111111111110 2554111111111111111111 2554111111111111111112 2554111111111111111113 2554111111111111111114 2554111111111111111115 2554111111111111111116 2554111111111111111117 2554111111111111111118 2554111111111111111119 25541111111111111111100 25541111111111111111101 25541111111111111111102 25541111111111111111103 25541111111111111111104 25541111111111111111105 25541111111111111111106 25541111111111111111107 25541111111111111111108 25541111111111111111109 25541111111111111111110 25541111111111111111111 25541111111111111111112 25541111111111111111113 25541111111111111111114 25541111111111111111115 25541111111111111111116 25541111111111111111117 25541111111111111111118 25541111111111111111119 255411111111111111111100 255411111111111111111101 255411111111111111111102 255411111111111111111103 255411111111111111111104 255411111111111111111105 255411111111111111111106 255411111111111111111107 255411111111111111111108 255411111111111111111109 255411111111111111111110 255411111111111111111111 255411111111111111111112 255411111111111111111113 255411111111111111111114 255411111111111111111115 255411111111111111111116 255411111111111111111117 255411111111111111111118 255411111111111111111119 2554111111111111111111100 2554111111111111111111101 2554111111111111111111102 2554111111111111111111103 2554111111111111111111104 2554111111111111111111105 2554111111111111111111106 2554111111111111111111107 2554111111111111111111108 2554111111111111111111109 2554111111111111111111110 2554111111111111111111111 2554111111111111111111112 2554111111111111111111113 2554111111111111111111114 2554111111111111111111115 2554111111111111111111116 2554111111111111111111117 2554111111111111111111118 2554111111111111111111119 25541111111111111111111100 25541111111111111111111101 25541111111111111111111102 25541111111111111111111103 25541111111111111111111104 25541111111111111111111105 25541111111111111111111106 25541111111111111111111107 25541111111111111111111108 25541111111111111111111109 25541111111111111111111110 25541111111111111111111111 25541111111111111111111112 25541111111111111111111113 25541111111111111111111114 25541111111111111111111115 25541111111111111111111116 25541111111111111111111117 25541111111111111111111118 25541111111111111111111119 255411111111111111111111100 255411111111111111111111101 255411111111111111111111102 255411111111111111111111103 255411111111111111111111104 255411111111111111111111105 255411111111111111111111106 255411111111111111111111107 255411111111111111111111108 255411111111111111111111109 255411111111111111111111110 255411111111111111111111111 255411111111111111111111112 2

panel (21) for terminating the electrical power supply to the bodies in the case of any emergency.

The drawbacks of the apparatus disclosed in our earlier Indian Patent No. 209817 are listed below:

1. the apparatus is not suitable for depositing thinner coatings on large area surfaces;
2. the apparatus is not suitable for depositing coatings on thin foils, sheets and wires;
3. the apparatus is suitable for depositing thicker coatings (85 to 95 microns as illustrated in Example 1 and Example 2 described in Indian Patent No. 209817) that possesses quite rough surface finish. Thereby the surface cleaning ability is poor and prone to dust accumulation;
4. the apparatus is not suitable for production scale as it is merely batch type processing based on the design of the electrolytic bath and also by the way that the bodies to be coated are arranged in the bath, which consumes a lot of time for fixing the bodies to be coated; and
5. the apparatus works with only two-phase electrical energy and leaves the third phase unutilized, therefore leading to electrical imbalance in the electrical mains.

Hence, it can be seen that there exists a need for providing a process for depositing uniform, thin films on sheets, foils and wires so as to enhance surface finish, thermal and electrical insulation, chemical inertness, surface cleaning ability, anti-dust sticking and to have good scratch resistance as well as depositing in a continuous manner and also an apparatus for carrying out the process.

#### SUMMARY OF THE INVENTION

Therefore, the main object of the present invention is to propose a process for depositing uniform, adherent, thin ceramic films on sheets, foils and wires in a continuous manner without any interruption.

Another object of the present invention is to propose a process for protecting the sheets, foils and wires in particular made of aluminum and its alloys to protect them against thermal, chemical, electrical and environmental reactions.

Still another object of the present invention is to propose a process for depositing uniform, adherent, thin ceramic films on sheets, foils and wires which is simple and economical.

Another object of the present invention is to propose an apparatus for carrying out the process for depositing uniform, adherent, thin ceramic films on sheets, foils and wires on a rapid production scale.

Yet another object of the present invention is to propose an apparatus for carrying out the process without having a transformer in the electrical circuit so that the electrical waveforms modified by thyristors are not distorted and therefore the coatings deposited are more uniform and adherent.

Still another object of the present invention is to propose an apparatus for carrying out the process wherein all three-phases of the power supply are properly used for coating deposition so that production rates are higher and electrical imbalances are minimized.

The above objects of the present invention are achieved by providing a process involving electro-thermal and electro-chemical oxidation of bodies in the form of sheets, foils or wires that continuously move in an alkaline electrolytic solution. In its broadest term, the present invention provides a new process for continuously electrolytically oxidizing metallic sheets, foils and wires.

#### BRIEF DESCRIPTION OF THE DRAWINGS

The present invention will be more fully understood from the following description taken in conjunction with the accompanying drawings wherein:

FIG. 1 represents a front view of a coating apparatus for carrying out the process disclosed in the prior art Indian patent;

FIG. 2 represents a front view of a main control panel for carrying out the process disclosed in the patent;

FIG. 3 represents a front view of a remote control panel for carrying out the process disclosed in the patent; and

FIG. 4 represents a schematic diagram of an embodiment of the apparatus of the present invention.

#### BRIEF DESCRIPTION OF THE INVENTION

Accordingly, the present invention provides an apparatus for continuously forming thin ceramic coatings on metal sheets, foils or wires (hereafter collectively referred to as metallic web). The apparatus comprises a reaction chamber (101) made up of a mild steel tank lined, both inside and outside, with Fibre Reinforced Plastic (FRP) for enhanced safety and to avoid any leakage of electrical energy. The reaction chamber (101) is capable of containing an alkaline electrolytic solution (102) tetrasilicate in de-ionized or distilled water. The reaction chamber (101) is provided with perforated nylon sheets (103), the sheets being attached to each other at each corner and being removably fixed and placed along the longitudinal walls of the reaction chamber (101). The nylon sheets (103) are also provided with three nylon bar guides (104) as well as three copper rods (105) that are able to rotate freely. Each of the copper rods (105) has a circular geometry and is separately connected to the R, Y and B phases of power supply, by high conductivity copper clamps (108) having a circular inner geometry. Each phase (R, Y and B Phases) is provided with two back-to-back thyristors (106) connected in parallel. The outputs of the thyristors (106) are connected to each of the copper rods (105) using three current transformers (CTs) (107). Three collecting nylon rods (109), each of which is capable of rotation by a drive means (110), are provided for collecting the metallic web after it is coated. The nylon rods (109) are attached at the top left portion of the nylon sheets (103). The chamber (101) also has an inlet (111) for the electrolyte provided at the bottom of the reaction chamber (101) and two outlets (112) for the electrolyte provided on the opposite side relative to the inlet side at the top of the reaction chamber (101).

By changing the location of the freely rotating nylon bars guides (104), either vertically or horizontally in the bath, it is possible to change the total surface area of the metallic web being coated without changing the basic design of the reaction chamber. This can be done by using the perforated nylon sheets (103) which permit the accommodation of more nylon bar guides (104) so that the webs to be coated can be passed in a zigzag manner to increase the residence time of the bodies in the bath, thus increasing the contact area of the metallic web which is to be coated with the electrolyte without necessitating any other design changes to the reaction chamber (101). Thereby, the overall productivity increases significantly and the rated power of the equipment is fully utilized. The coated web can be moved through the electrolyte solution (102) by drive means acting on one or more of the copper rods (105). Collecting nylon rods (109) are capable of rotating at a preset rpm by employing a drive (110) attached to the outer frame of reaction chamber (101) with the help of a conventional reduction gear system. The linear velocity of the metallic web, or in other words the residence time of the web inside the bath, is controlled by adjusting the rpm of the drive.

According to another feature of the invention, there is provided a process for forming coatings on metal sheets, foils or wires (hereafter collectively referred to as metallic web).

The process comprises immersing at least three metallic webs selected from the reactive group of metals on which coatings have to be effected, in an alkaline electrolytic solution having a pH>12 and conductivity>2 millimhos, the electrolytes solution comprising potassium hydroxide, sodium tetrasilicate in de-ionized or distilled water contained in the reaction chamber (101) of the device as defined above. Wave multiphase alternating current is passed across the web by the back-to-back thyristors connected in parallel for a period based on the desired thickness of the coatings to be achieved. The current being supplied to the web is slowly increased until the required current density is achieved. The flow of the electrolyte is in the direction perpendicular to the direction of the moving metallic web in such a way that cross flow is attained for effective heat dissipation in the reaction chamber. The current is maintained at the same level throughout the process. The electric potential is further increased gradually to compensate for the increasing resistance of the coating when visible arcing at the surface of the immersed regions of the said web is noticed. The composition of the electrolyte is regulated by measuring its pH and conductivity during the process by conventional methods. The temperature of the electrolyte is maintained between the range of 4° C. to 50° C. and the electrolyte is kept in continuous circulation throughout the process. The coated web is removed by taking out the perforated nylon sheets from the reaction chamber (101).

The electrolytic solution (102) enters the reaction chamber (101) through the inlet (111) provided at the bottom of reaction chamber (101) and leaves the reaction chamber (101) through two outlets (112) provided on the opposite side relative to inlet side at the top of the reaction chamber (101). A three-phase electrical power is supplied through two back-to-back thyristors (106) connected in parallel provided for each phase (R, Y and B Phases), which are employed for modifying the current and voltage waveforms. All the three phases of modified wave electrical power is then passed through three metallic webs to be coated leading to enhanced production rate and minimized electrical imbalances in the electrical mains. Three current transformers (CTs) (107) consisting of x, y, z and common point c are provided to the R, Y and B phases in the manner to separately measure the magnitude of current flowing in the three phases and the resultant averaged electrical signal is fed to the thyristor block (106) so that the constant current supply is provided throughout the coating deposition process.

In a preferred embodiment of the invention, the electrolyte used may contain potassium hydroxide and sodium tetrasilicate in a preferred ratio of 2:1. The web on which the deposition is to be made may be selected from the reactive group of metals consisting of Al, Ti, Mg, Zr, Ti, Be, Ge, Ca, Te, Hf, and V and their binary, ternary and multi-constituent alloys with elements like Cu, Zn, Mg, Fe, Cr, Co, Si, Mn, Al, Ti, Mg, Zr, Ta, Be, Ge, Ca, Te, Hf, V, and W.

The material of the web is allowed to move at a preset velocity by adjusting the speed of the drive (110). The linear velocity of the web is calculated based on the residence time in the bath required for depositing the required film thickness. The flow of electrolyte is in the direction perpendicular to the direction of the moving web in such a way that a cross flow is attained for effective heat dissipation in the reaction chamber (101). The flow rate of electrolyte in liters per minute is calculated based on the surface area of the web being coated in such a way that the ratio of total surface area (in sq. cm) to the flow rate (in liters per minute) is maintained between 0.1 and 1.2 so as to maintain a constant temperature of the bath. The electrolyte is circulated through an air cooled heat exchanger system so that the bath temperature is maintained

constant. Accordingly, the cooled electrolyte enters the reaction chamber (101) through an inlet (111) provided at its bottom, and the hot electrolyte leaves through outlets (112) at the top of the chamber. Two back-to-back thyristors connected in parallel provided for each phase (R, Y and B Phases) are employed both for modifying the current and voltage waveforms. The firing angle of the thyristors is based on the feedback signal obtained by collecting the average value of electrical current passing through each individual phase and using this average value as a feedback signal thus maintaining the constant current supply throughout the process. The modified wave electrical power is passed through at least three webs to be coated or multiples of three webs. The magnitude of current is based on the contact surface area of the body to be coated with the electrolyte. The total time of power supply is based on the total length (in meters) of the web (sheet, foil or wire) being coated divided by the linear velocity (meters/seconds) of the body in the bath.

By carrying out the process as described above, it is possible to obtain thin films of predetermined thickness in the range of 0.25 to 10 microns on sheets and foils having a wide range of widths from 10 cm to 500 cm, and wires of varying diameters from 0.02 cm to 2.0 cm and over a total length of several kilometers without any interruption, providing superior quality coating and enhanced production rates. The thin films thus obtained by employing the above-described process have exhibited glossy surface finishes, thermal and electrical insulation, chemical-inertness, surface cleaning ability, anti-dust sticking and good scratch resistance. Further, the thin films produced by this method are more adherent, smooth and uniform than the coatings produced in the prior art.

The details of the invention are given in the Examples given below which are provided for illustrating the invention and therefore should not be construed to limit the scope of the present invention.

#### Example 1

Three high purity aluminum foils of each 68 mm width, 30 micron thickness and 500 meter long dimension were connected to an output of a power supply. A total surface area in contact with an electrolyte was adjusted to be about 2100 cm<sup>2</sup> and a three-phase current of 210 A was passed through each web and maintained constant throughout the process. The surface area of the web in contact was adjusted by adjusting the location of nylon bars. Electrolyte containing potassium hydroxide and sodium tetrasilicate in a ratio of 2:1 (4 g/l potassium hydroxide and 2 g/l sodium tetrasilicate) mixed in de-ionized water was circulated through the reaction chamber throughout the process. The electrolyte flow rate of 250 liters per minute was maintained throughout the process. The rpm of the drive is set at 550 revolutions per minute so that a linear velocity of 2.2 m/min was maintained constant throughout the process. The process was continued for a total duration of 3 hrs 50 minutes to coat a total foil of length equal to 1.5 kilometers resulting in a deposition of 0.5 micron thick film on a total surface area of 1,020,000 square centimeters. The films formed were found to have excellent adhesion, glossy surface finish, and high degree of uniformity without leaving any uncoated areas without any surface defects. In addition, the deposited films were found to be decorative, thermally and electrically insulative, chemically inert, exhibited easy surface cleaning ability, anti-dust sticking and were environmentally non-reactive.

#### Example 2

Nine electrical grade aluminum spools, each containing wires of 4 mm diameter, and 1000 meter (1 kilometer) long

dimension were connected to an output of a power supply. A total surface area in contact with an electrolyte is adjusted to be about 2260 cm<sup>2</sup> and a three-phase current of 225 A was passed through each web and maintained constant throughout the process. The surface area of the web in contact was adjusted by adjusting the location and also by placing more nylon bars. In order to avoid the lateral movements, the wire was passed through individual non-metallic guides attached to nylon bars so that any possibility of electrical short circuit was completely eliminated. Electrolyte containing potassium hydroxide and sodium tetrasilicate in the ratio of 2:1 (4 g/l potassium hydroxide and 2 g/l sodium tetrasilicate) mixed in de-ionized water was circulated through the reaction chamber throughout the process. The electrolyte flow rate of 1200 liters per minute was maintained throughout the process. The rpm of the drive was set at 550 revolutions per minute so that a linear velocity of 2.7 m/min was maintained constant throughout the process. The process was continued for a total duration of 6 hrs to coat a total foil of length equal to 9 kilometers. The average film thickness was found to be 1.0 micron. The films formed were found to have excellent adhesion, glossy surface finish, high degree of uniformity without leaving any uncoated areas, without any surface defects. In addition, the deposited films were found to be decorative, thermally and electrically insulative, chemically inert, exhibited easy surface cleaning ability, anti-dust sticking and were environmentally non-reactive.

### Example 3

Three aluminum alloy sheets having 136 mm width, 0.2 mm thickness have been subjected to similar processes as described in Example 1. The surface area of the web in contact with electrolyte was adjusted by adjusting a location of nylon bars. Electrolyte containing potassium hydroxide and sodium tetrasilicate in the ratio 2:1 (4 g/l potassium hydroxide and 2 g/l sodium tetrasilicate) mixed in de-ionized water was circulated through the reaction chamber throughout the process. The electrolyte flow rate of 250 liters per minute was maintained throughout the process. The rpm of the drive is set so that a linear velocity of 0.22 m/min is maintained constant throughout the process. The process was continued for a total duration of 3 hrs 50 minutes to coat a total foil of length equal to 1.5 kilometers resulting in deposition of 5 micron thick film on a total surface area of 1,020,000 square centimeters. The applied current, electrolyte flow rate and treatment time were calculated accordingly and the films of 5 micron thickness were successfully deposited. The films were found to be uniform, homogeneous, environmentally non-reactive, and electrically and thermally insulative. Furthermore, the films formed have exhibited good scratch resistance as well.

It is apparent to a person reasonable skilled in the art that modifications and changes can be made within the spirit and scope of the present invention. Accordingly, such modifications and changes are also covered within the scope of the present invention.

### ADVANTAGES OF THE INVENTION

1. The films obtained by the process using the apparatus of the present invention are uniform, exhibit glossy surface and are well bonded with the substrate.
  2. The sheets, foils and wires prepared by the process using the apparatus of the present invention can be directly used for decorative, automobile, space, mild corrosion, anti-dust sticking, glossy/matt finishing, insulation, and mild chemical resistant applications.
- 10
3. The process using the apparatus described permits the continuous coating formation without intermediately stopping the process on the web of several kilometers long.
  4. The process using the apparatus disclosed in the present invention permits the rapid rate formation of thin films on sheets, foils and wires.
  5. The overall cost of film deposition on the web offered by the present invention is negligibly low compared to the coatings produced by the process hitherto known.
  6. The web, in widely differing widths and thicknesses in the case of sheets and foils, or with different diameters in the case of wires, can be treated without any design changes in the apparatus disclosed in the present invention.
- 15
- It is to be noted that the present invention is susceptible to modifications, adaptations and changes by those skilled in the art. Such variant embodiments employing the concepts and features of this invention are intended to be within the scope of the present invention, which is further set forth under the following claims.
- We claim:
1. An apparatus for continuously forming thin ceramic coatings on metallic web, the apparatus comprising:  
a reaction chamber; and  
perforated sheets placed in the reaction chamber; and  
a plurality of bar guides placed in the reaction chamber,  
wherein the location of the bar guides is changeable  
using the perforated sheets, which permit accommoda-  
tion of the bar guides, to change a total surface area of the  
metallic web being coated.
  2. The apparatus of claim 1, wherein the reaction chamber  
is capable of containing an alkaline electrolytic solution.
  3. The apparatus of claim 1, wherein the perforated sheets  
are perforated nylon sheets.
  4. The apparatus of claim 1, wherein the perforated sheets  
are attached to each other at each corner and are removably  
fixed and placed along longitudinal walls of the reaction  
chamber.
  5. The apparatus of claim 1, wherein the bar guides are  
nylon bar guides.
  6. The apparatus of claim 1, further comprising conductive  
rods that are able to rotate freely, each of the conductive rods  
having a circular geometry and being separately connected to  
an R, Y, or B phase of a power supply by high conductivity  
clamps having a circular inner geometry, each phase (R, Y or  
B Phase) being provided with two back-to-back thyristors  
connected in parallel, the outputs of the thyristors being con-  
nected to each of the conductive rods using current transfor-  
mers (CTs).
  7. The apparatus of claim 6, wherein the conductive rods  
and high conductivity clamps and copper rods and copper  
clamps.
  8. The apparatus of claim 1, further comprising collecting  
rods provided for collecting the metallic web after being  
coated, wherein each collecting rod is capable of rotation and  
is attached at the top portion of the sheets.
  9. The apparatus of claim 8, wherein the collecting rods are  
collecting nylon rods.
  10. The apparatus of claim 1, further comprising an inlet  
for the electrolytic solution provided at the bottom of the  
reaction chamber and two outlets for the electrolytic solution  
provided on the opposite side relative to inlet side at the top of  
the reaction chamber.
  11. An apparatus for continuously forming thin ceramic  
coatings on metallic web, the apparatus comprising: a reaction  
chamber, wherein the reaction chamber is capable of
- 20
- 25
- 30
- 35
- 40
- 45
- 50

**11**

containing an alkaline electrolytic solution, the reaction chamber being provided with perforated nylon sheets, the nylon sheets being attached to each other at each corner and being removably fixed and placed along the longitudinal walls of the reaction chamber, the nylon sheets being provided with three nylon bar guides and three copper rods, wherein the copper rods are able to rotate freely, each of the copper rods having a circular geometry and being separately connected to an R, Y, or B phase of a power supply by high conductivity copper clamps having a circular inner geometry, each phase (R, Y or B Phase) being provided with two back-to-back thyristors connected in parallel, the outputs of the thyristors being connected to each of the copper rods using three current transformers (CTs), three collecting nylon rods provided for collecting the metallic web after being coated, wherein each collecting nylon rod is capable of rotation and is attached at the top portion of the nylon sheets, the reaction chamber also having an inlet for the electrolytic solution provided at the bottom of the reaction chamber and two outlets for the electrolytic solution provided on the opposite side relative to inlet side at the top of the reaction chamber.

**12.** The apparatus of claim **11**, wherein the reaction chamber is comprised of a mild steel tank lined both inside and outside with Fibre Reinforced Plastic (FRP).

**13.** The apparatus of claim **11**, wherein the electrolytic solution comprises potassium hydroxide and sodium tetrasilicate in de-ionized or distilled water.

**14.** The apparatus of claim **11**, wherein the metallic web is metal sheets, foils, or wires.

**12**

**15.** An apparatus for continuously forming thin ceramic coatings on metal sheets, foils or wires hereafter collectively referred to as metallic web, the apparatus comprising: a reaction chamber comprised of a mild steel tank lined both inside and outside with Fibre Reinforced Plastic (FRP), wherein the reaction chamber is capable of containing an alkaline electrolytic solution comprising potassium hydroxide and sodium tetra silicate in de-ionized or distilled water, the reaction chamber being provided with perforated nylon sheets, the nylon sheets being attached to each other at each corner and being removably fixed and placed along the longitudinal walls of the reaction chamber, the nylon sheets being provided with three nylon bar guides and three copper rods, wherein the copper rods are able to rotate freely, each of the copper rods having a circular geometry and being separately connected to an R, Y, or B phase of a power supply by high conductivity copper clamps having a circular inner geometry, each phase (R, Y, or B phase) being provided with two back-to-back thyristors connected in parallel, the outputs of the thyristors being connected to each of the copper rods using three current transformers (CTs), three collecting nylon rods provided for collecting the metallic web after being coated, wherein each collecting nylon rod is capable of rotation and is attached at the top portion of the nylon sheets, the reaction chamber having an inlet for the electrolytic solution provided at the bottom of the reaction chamber and two outlets for the electrolytic solution provided on the opposite side relative to the inlet side at the top of the reaction chamber.

\* \* \* \* \*